

# United States Patent [19]

Hage et al.

[11] Patent Number: 4,476,704

[45] Date of Patent: Oct. 16, 1984

[54] METHOD FOR PRODUCING FINNED TUBES

4,314,587 2/1982 Hackett ..... 138/38  
4,349,949 9/1982 Kritzer ..... 29/157.3 A

[75] Inventors: Manfred Hage, Ulm; Gerhard Schinkoth, Neu-Ulm, both of Fed. Rep. of Germany

802854 2/1951 Fed. Rep. of Germany .  
1767057 3/1958 Fed. Rep. of Germany .  
1126431 3/1962 Fed. Rep. of Germany .  
1776135 1/1970 Fed. Rep. of Germany .  
64924 5/1980 Japan ..... 72/274  
565027 10/1944 United Kingdom .  
1290588 9/1972 United Kingdom .

[73] Assignee: Wieland-Werke AG, Ulm, Fed. Rep. of Germany

[21] Appl. No.: 471,289

[22] Filed: Mar. 2, 1983

Related U.S. Application Data

[62] Division of Ser. No. 328,756, Dec. 8, 1981, Pat. No. 4,425,942.

Primary Examiner—Daniel C. Crane  
Attorney, Agent, or Firm—Ladas & Parry

[30] Foreign Application Priority Data

Dec. 24, 1980 [DE] Fed. Rep. of Germany ..... 3048959

ABSTRACT

[51] Int. Cl.<sup>3</sup> ..... B21C 1/00; B21D 53/06

A finned tube for a heat exchanger has an inner surface in which is provided raised portions which are in rows and extend in the longitudinal direction of the tube. The raised portions are arranged, within each row, at irregular intervals and each raised portion may either increase or decrease toward a radially inward tip. The raised portions may have a cross-section which is substantially triangular or trapezoidal or in the shape of a parallelogram and the lateral surfaces of the raised portions, together with the internal surfaces of the tube are roughened during drawing.

[52] U.S. Cl. ..... 72/276; 72/367; 29/157.3 A

In a process of making such a tube, an unhardened tube having a plurality of circumferentially disposed longitudinally extending fins is drawn through a die so as to subject the tube to a cross-sectional decrease of at least 50% to thereby fragment the fins to provide gaps between remaining raised portions of the fins.

[58] Field of Search ..... 72/276, 274, 467, 367; 29/157.3 A; 138/37-39; 165/133, 179, 183, 184

A drawing die for used in the process has an entry angle  $\alpha \geq 40^\circ$ .

[56] References Cited

12 Claims, 3 Drawing Figures

U.S. PATENT DOCUMENTS

1,728,016 9/1929 Staples ..... 72/276  
2,228,301 1/1941 Ditzel et al. ..... 72/276  
3,267,563 8/1966 Seaton ..... 29/157.3 A  
3,267,564 8/1966 Keyes ..... 29/157.3 A  
3,273,599 9/1966 Heeren .....  
3,402,767 9/1968 Bohdansky et al. ....  
3,612,175 10/1971 Ford et al. ..... 165/179  
3,750,709 8/1973 French ..... 29/157.3 A  
3,776,018 12/1973 French ..... 29/157.3 A  
3,910,085 10/1975 Biddell et al. ..... 72/467  
4,087,893 5/1978 Sata et al. ..... 29/157.3 A





Fig. 1



Fig. 2



Fig. 3

## METHOD FOR PRODUCING FINNED TUBES

This is a division of application Ser. No. 328,756 filed Dec. 8, 1981, now U.S. Pat. No. 4,425,942, issued July 26, 1983.

This invention relates to a finned tube for a heat exchanger.

In particular the present invention relates to a finned tube of the type having raised portions which are present on the inner surface of the tube and which are arranged in rows extending in the longitudinal direction of the tube and which possess lateral surfaces which also extend in the longitudinal direction of the tube.

A finned tube of the said type, as described in German Auslegeschrift No. 2,032,891, possesses raised portions on the inner surface of the tube which essentially have the shape of truncated pyramids. Although, compared to a smooth tube, a tube of this type presents advantages related to heat technology, because, for example when being operated as an evaporator, the heat transfer characteristics for the coolant can be improved through the generation of turbulence at the raised portions, the latter, and other factors, nevertheless necessitates a comparatively laborious procedure for the manufacture of a tube of this type, since it must be produced in two drawing steps, each of which is carried out over a mandrel provided with helical grooves, or with straight grooves.

An object of this invention is to provide a finned tube having internal raised portions, which, while possessing improved heat transfer characteristics, can at the same time be manufactured significantly more easily.

According to this invention there is provided a finned tube for a heat exchanger comprising a tube having an outer surface and an inner surface, raised portions provided on said inner surface which raised portions are arranged in rows extending in a longitudinal direction of the tube and which possess lateral surfaces which also extend in the longitudinal direction of the tube, said raised portions being arranged, within a row, at irregular intervals.

The object is thus achieved, according to the invention, by virtue of the fact that the raised features are arranged, within a row, at irregular intervals so that the generation of turbulence is significantly promoted by the irregular arrangement of the raised portions.

The width of each raised portions may either increase or decrease in a smooth manner, in the radially inward direction towards the tips of the raised portions.

The ends of the raised portions may be expediently rounded off, the raised portions having, in particular, a triangular cross-section, or a flattened cross-section.

The lateral surfaces of the raised portions preferably converge at each end, to form an edge.

The raised portions may each have, in longitudinal section, an approximation, to the shape of a trapezium, or the shape of a parallelogram which each face in the same direction, that is to say, acutely inclined edges point in one direction of the tube, whilst obtusely inclined edges point in the other direction.

It is advisable, in order to multiply the number of bubble nuclei of a coolant in use, to form the lateral surfaces and the ends of the raised portions, and the inside surfaces of the tube between the raised portions, so that they are roughened.

An additional contribution may be made to improve the heat transfer in the outward direction when the gaps

between individual raised features extend as far as the root circle of the raised features, and when the outside surface of the finned tube is slightly corrugated.

A process for manufacturing the finned tube according to the invention is a further aspect of the invention.

The process provides an initial tube, having a plurality of circumferentially disposed internal fins each extending in the longitudinal direction of the tube, work-hardening the tube in a drawing die and subjecting, during drawing, the tube to a diameter-reduction using a cross-sectional decrease of at least 30%, and preferably 35 to 50%, accompanied by necking of the tube.

In this context, the term "necking" should be understood as meaning that the work-hardened tube in the drawing die is initially drawn in with a small radius of curvature, and is subsequently bent back, in the opposite direction, with a radius of curvature which is equally small.

In this context, the undermentioned quantity is defined as the cross-sectional decrease:

$$\frac{\text{Area of the cross-section of the tube before the diameter-reducing draw} - \text{Area of the cross-section of the tube after the diameter-reducing draw}}{\text{Area of the cross-section of the tube before the diameter-reducing draw}}$$

As a result of severe necking and the heavy diameter-reducing draw, the original longitudinal fins tear, and irregularly arranged raised portions are formed. At the same time, rough surfaces are obtained on the inside of the tube.

In contrast to the customary sequence of approximately 4 to 6 drawing steps, only two drawing steps preferably have to be carried out according to the process in accordance with the invention, an approximately true-to-scale reduction of the tube being achieved without using a profiled internal mandrel. In addition, it is possible to obtain smaller wall thickness than was previously the case. The grain size of the starting tube plays a decisive part in the formation of the tears; the coarser the grain, the greater is the susceptibility to tearing and the deeper are the tears. The grain size  $D_K$  of the starting tube is at least 0.100 mm, preferably 0.150 to 0.300 mm.

It is, moreover, advisable to use an unhardened tube, preferably an extruded tube, as the starting tube. In a preferred embodiment of the invention, the Vickers hardness HV of the work-hardened tube is thus 200 to 250% of the Vickers hardness of the unhardened starting tube.

The invention further relates to a drawing die for carrying out the process according to the invention.

The drawing die is characterised by an entry angle  $\alpha \geq 40^\circ$  and by a sharp edge at the transition from the conical portion to the cylindrical portion. An entry angle  $\alpha = 45^\circ$  to  $50^\circ$  is preferred.

The invention will now be described, by way of example, with reference to the accompanying drawings, in which:

FIG. 1 shows a longitudinal section of a finned tube in accordance with the invention;

FIG. 2 shows a transverse section through the finned tube of FIG. 1; and

FIG. 3 shows a longitudinal section through a drawing die of an aspect of the invention.

The finned tube 1 shown in FIGS. 1 and 2 has internally raised fin portions 2 separated by gaps 3, the por-

tions 2 being arranged in rows extending in the tube longitudinal direction and being irregularly spaced in each row. The tube is formed by diameter-reducing drawing of a work-hardened tube previously unhardened and provided with internal longitudinal fins, and as a result of the diameter-reducing draw the longitudinal fins undergo tearing resulting in the irregularly arranged fin portions 2 separated by the gaps 3.

As shown in FIG. 2, the internally raised portions 2 retain the original shape of the longitudinal fins, that is, lateral surfaces 4 of the raised portions 2 extend in the longitudinal direction of the tube, and the width of each raised portion 2 in a circumferential direction, smoothly decreases in a radially inward direction towards a tip 5 of each raised portion.

Referring to FIG. 1, the raised portions 2 essentially have the shape of parallelograms, which all face in the same direction. The raised portions 2, in the longitudinal direction have edges 6, 8 which form an acute angle with the drawing direction of the tube, indicated by arrow 7.

In the present exemplary embodiment, the gaps 3 extend as far as the root circle 9 of the raised portions 2 but the rough formation of the lateral surfaces 4 and of the inner surfaces 14 of the tube, between the raised features 2, is not illustrated.

In alternative embodiments of the invention the width of each raised portion in a circumferential direction smoothly increases in a radially inner direction towards a tip 5 of each raised portion. Furthermore, the tips 5 of the raised portions, instead of being rounded, may be flattened off. In yet another alternative embodiment, the raised portions 2 each have a longitudinal cross-section which exhibits approximately the shape of a trapezium. Furthermore, the outer surface of the finned tube may, instead of being smooth, be slightly corrugated.

The formation of the tears in the longitudinal fins will now be explained with reference to FIG. 3. The initial unhardened tube, provided with circumferentially disposed longitudinal fins is driven into a drawing die 10 in the direction of arrow headed lines 7. Because of a sharp edge 13, in the die entry the tube is bent through an angle  $\alpha$  in the range of 45° to 50°. The tears forming gap 3 are formed while the tube is conically shaped by a portion 11 of the die and the tube is necked down to the cylindrical portion 12. Because of the severe deformation of the tube material, on drawing further, the tears are spread further as a result of the elongation of the tube.

An actual example of a tube in accordance with this invention will now be described.

#### EXAMPLE

Extruded copper tubes having an outside diameter of 28 mm and having 20 internal fins were available as starting tubes. The grain size  $D_K$  was 0.150 mm. These extruded tubes were work-hardened by drawing-down to tubes having the following data:

|                      |         |
|----------------------|---------|
| Outside diameter:    | 23 mm   |
| Wall thickness:      | 1.20 mm |
| Fin Height:          | 1.80 mm |
| Vickers Hardness HV: | 103     |

The work-hardened tubes were drawn in two steps:

|           |                                          |         |
|-----------|------------------------------------------|---------|
| 1st Draw: | Diameter of the drawing die:             | 19.1 mm |
|           | Entry angle $\alpha$ of the drawing die: | 48°     |
|           | Outside diameter of the tube:            | 17.2 mm |

-continued

|   |           |                                          |         |
|---|-----------|------------------------------------------|---------|
| 5 | 2nd Draw: | Wall thickness of the tube:              | 1.00 mm |
|   |           | Fin height:                              | 1.45 mm |
|   |           | Decrease in cross-section:               | 36%     |
|   |           | Diameter of the drawing die:             | 13.5 mm |
|   |           | Entry angle $\alpha$ of the drawing die: | 48°     |
|   |           | Outside diameter of the tube:            | 12.0 mm |
|   |           | Wall thickness of the tube:              | 0.80 mm |
|   |           | Fin height:                              | 1.10 mm |
|   |           | Decrease in cross-section:               | 45%     |

The internal fins of the tubes, treated in this way, were torn down to the tube internal root material.

An extruded tube may be used as the initial tube and the Vickers hardness of the work-hardened tube is 200 to 250% of the Vickers hardness of the unhardened, initial tube.

The advantages of tubes made by the present invention in relation to heat technology, becomes evident when, for example, they are employed in coaxial evaporators. Coaxial evaporators usually consist of one or more inner tubes, over which a jacket-tube is pushed. The water flows in the space between the inner tubes and the jacket-tube, and the coolant which is fed in a counter-direction to the water, evaporates in the inner tubes.

The data describing a coaxial evaporator, using the finned tubes according to the invention as inner tubes, and the data relating to a coaxial evaporator using conventional five-rayed star-section tubes having the designation 5-12-08 (five-rayed, outside diameter 12.0 mm, wall thickness 0.80 mm) are summarised in the Table which follows:

| 35 | Coaxial evaporator using inner tubes according to the invention | evaporator using star-section inner tubes |
|----|-----------------------------------------------------------------|-------------------------------------------|
| 40 | Jacket-tube (mm) 35 × 1                                         | 35 × 1                                    |
|    | Inner tube:                                                     |                                           |
|    | Outside diameter (mm) 12.0                                      | 12.0                                      |
|    | Wall thickness (mm) 0.8                                         | 0.8                                       |
|    | Number of inner tubes 3                                         | 3                                         |
| 45 | Coil diameter (mm) 450 ± 5                                      | 450 ± 5                                   |
|    | Number of turns 3.5                                             | 3.5                                       |
|    | The operating data were:                                        |                                           |
|    | Evaporation temperature: $t_o = 0^\circ \text{C}$ .             |                                           |
|    | Water inlet temperature: $t_{w1} = 12^\circ \text{C}$ .         |                                           |
|    | Coolant: R 22                                                   |                                           |

It was found that the coaxial evaporator using the inner tubes according to the invention exhibited a capacity which was approximately 20% higher than that of a coaxial evaporator using star-section inner tubes, for identical external geometries (identical structural volume, identical weight), and the same pressure-drop on the water side.

We claim:

60 1. A process for manufacturing a finned tube having a circumferentially disposed plurality of internal fins, each fin extending in the longitudinal direction of the tube and being discontinuous therealong such that each fin is made up of a plurality of fin portions, said process comprising the steps of:

providing a tube having a plurality of internal fins, each fin extending in the longitudinal direction of said tube and being continuous therealong,

moving said tube through a drawing die so that it undergoes a diameter reduction associated with a decrease in cross sectional area of at least thirty percent and so that said fins are torn into a series of torn portions extending in longitudinal rows along the tube,

said torn portions being produced solely by said diameter reduction of said tube, and further drawing the tube so as to longitudinally separate the torn portions and produce a finned tube 10 having said plurality of fin portions.

2. A process as claimed in claim 1, wherein the decrease in the cross-section during the diameter-reducing draw is 35 to 50%.

3. A process as claimed in claim 1, wherein only two 15 drawing steps are performed.

4. A process as claimed in claim 1, wherein the starting tube to be drawn possesses a large grain size.

5. A process as claimed in claim 4, wherein the grain size of the tube is at least 0.100 mm.

6. A process as claimed in claim 5, wherein the grain size is 0.150 to 0.300 mm.

7. A process as claimed in claim 1, wherein the tube is initially unhardened.

8. A process as claimed in claim 7, wherein an extruded tube is used.

9. A process as claimed in claim 7, wherein the Vickers hardness of the tube is 200 to 250% of the Vickers hardness of the unhardened tube.

10. A process as claimed in claim 1, wherein said drawing die possesses a conical portion extending to a cylindrical portion with an entry angle  $\alpha \geq 40^\circ$ , and a sharp edge at the transition from the conical portion extending to a cylindrical portion.

11. A process as claimed in claim 10, wherein the entry angle is in the range  $45^\circ$  to  $50^\circ$ .

12. The process claimed in claim 1 in which the tube is work hardened when it is moved through the drawing die.

\* \* \* \* \*